

## UNITED STATES PATENT OFFICE

2,082,719

## HARD METAL ALLOY

Alan Richard Powell and Ernest Robert Box, London, England, assignors to Johnson Matthey & Company, Limited

No Drawing. Original application October 4, 1933, Serial No. 692,219. Divided and this application June 1, 1936, Serial No. 82,980. In Great Britain October 11, 1932

## 6 Claims. (Cl. 75—172)

This application is a division of our copending parent application Serial No. 692,219, filed October 4th, 1933, and is filed in response to a final requirement of division therein. Said application has matured into Patent No. 2,070,451, granted Feb. 9, 1937.

This invention relates to the manufacture and production of hard metal alloys especially useful for tipping the points of gold nibs and the points of compass needles. Such alloys in addition to great hardness must be resistant to tarnishing and to corrosion by dilute solutions of the common acids and alkali, must have a high resistance to wear, must be capable of being readily soldered onto gold and onto copper and iron base metal alloys and must be sufficiently tough not to chip or splinter when subjected to grinding, polishing or slitting operations. At one time native grains of osmiridium were solely used for these purposes but the supplies of this natural product are not sufficiently uniform in size and shape; hence numerous alloys have been made for this purpose by melting together some or all of the constituents of osmiridium with other metals of the platinum group with or without the addition of base metals to increase the hardness. Efforts to convert native osmiridium into grains suitable for tipping nibs by melting the alloy alone or with the addition of other constituents have so far not produced grains of a quality equal to that of native grains.

We have now found that suitable alloys for the said purposes may be made by melting native or synthetic osmiridium (by which is meant throughout the specification and claims an alloy of 40 to 60 per cent of osmium; 60 to 40 per cent of iridium and 0 to 20 per cent of ruthenium) or of osmium and/or ruthenium together with an element of the group consisting of cobalt and nickel (3 to 25 per cent) and boron (0.1 to 5 per cent). The alloy should contain at least 75 per cent of osmiridium or of osmium and/or ruthenium.

In making the alloys the constituents may be mixed together in the form of powders or small grains and the mixture melted in a suitable furnace as, for example, an electric furnace of the induction, resistance or arc type. We prefer however to add the boron in the form of an alloy with the element of the group consisting of cobalt and nickel for example as cobalt boride.

The best alloys are those the proportions of the

components of which are within the following ranges:—

|                                                               | Per cent |
|---------------------------------------------------------------|----------|
| Osmiridium or an equivalent amount of osmium and/or ruthenium | 75 to 95 |
| Cobalt and/or nickel                                          | 5 to 25  |
| Boron                                                         | 0.5 to 3 |

## Example 1

|                                                                                                  | Per cent |
|--------------------------------------------------------------------------------------------------|----------|
| Native osmiridium                                                                                | 80       |
| Cobalt                                                                                           | 19.5     |
| Boron, the boron being added in the form of a cobalt boron alloy containing 10 per cent of boron | 0.5      |

## Example 2

|                   | Per cent |
|-------------------|----------|
| Native osmiridium | 90       |
| Cobalt            | 9        |

Boron, the boron being added in the form of cobalt boride

We claim:

1. A hard metal alloy of the kind defined consisting of 75 to 94.5% of at least one metal of the group consisting of osmiridium, osmium and ruthenium, 3 to 25% of at least one metal of the group consisting of cobalt and nickel, and 0.1 to 5% boron.

2. A hard metal alloy of the kind defined consisting of 75 to 94.5% of at least one metal of the group consisting of osmiridium, osmium and ruthenium, 3 to 25% cobalt, and 0.1 to 5% boron.

3. A hard metal alloy of the kind defined consisting of 75 to 94.5% of at least one metal of the group consisting of osmiridium, osmium and ruthenium, 3 to 25% of a metal of the group consisting of cobalt and nickel, and 0.1 to 5% boron added as a boride of the said metal of the group consisting of cobalt and nickel.

4. A hard metal alloy of the kind defined consisting of 75 to 94.5% of osmiridium, 3 to 25% of at least one metal of the group consisting of cobalt and nickel, and 0.1 to 5% boron.

5. A hard metal alloy of the kind defined consisting of 80 to 90% of osmiridium, 19.5% to 9% of cobalt, and 0.5 to 1% of boron.

6. A hard metal alloy of the kind defined consisting of 80% of osmiridium, 19.5% of cobalt and 0.5% boron.

ALAN RICHARD POWELL.  
ERNEST ROBERT BOX.